

# UNITED STATES PATENT OFFICE.

ALEXANDER H. EGE, OF MECHANICSBURG, PENNSYLVANIA.

## ARTIFICIAL FUEL.

No. 913,713.

Specification of Letters Patent.

Patented March 2, 1909.

Application filed November 8, 1907. Serial No. 401,321.

*To all whom it may concern:*

Be it known that I, ALEXANDER H. EGE, a citizen of the United States, residing at Mechanicsburg, in the county of Cumberland, State of Pennsylvania, have invented 5 certain new and useful Improvements in Artificial Fuel, of which the following is a specification.

The object of this invention is to produce 10 a fuel, having as a base alcohol and coal dust, which shall be suitable for handling, and which shall have great heat producing properties.

Fuel made in accordance with my invention 15 consists of a more or less friable compound of a consistency somewhat less than that of semi-pulverized bituminous coal, and it is very inflammable. The alcohol used in making the fuel is preferably denatured 20 alcohol on account of its cheapness, and this is mixed with the fine powder of coal which is known as coal dust, coal slack or screenings. The coal dust may be that from an- 25 thracite, bituminous or lignite coal, or from peat.

While the basic elements of my fuel are coal dust and alcohol I find it advisable to add other ingredients to adapt the fuel to special uses and to secure certain desirable 30 qualities which fit it for those uses. The proportions of the ingredients furthermore vary within certain limits, according to the particular qualities that are necessary for the particular use desired.

When mixed in the proportions of 4 parts of coal dust to 1 part of alcohol my fuel is in such form as to be adapted for transportation, being sufficiently solid for that purpose. When however it is intended for use in the 40 immediate neighborhood of the place of manufacture the ingredients may be combined in the proportions 2 to 1. When it is desired to solidify the mixture into lumps for more ready transportation to a distance, I 45 add a binder thereto consisting of cement or a flour paste derived from the ground grain of wheat, rye, corn, rice or other starch producing material. In such case the pasty consistency of the flour is produced by mixing 50 it with the alcohol which is to be used more or less diluted, and this is done before mixing the alcohol with the coal dust. The composition after being mixed is pressed into blocks or lumps and is dried. I find a good 55 proportion in this case to be 1 part of alcohol, 1 of flour and 4 parts of coal dust. The

material does not burn so rapidly when the flour or cement is mixed therewith, as above stated, but this addition secures a more solid article which may be more easily 60 shipped. In case I require a still more solid compound, but somewhat diminished combustibility, I substitute for my flour paste that of cement, either hydraulic or Portland, with an addition of water, observing the proportions of 1 part cement, 2 parts of water, 65 2 parts of alcohol, and 5 parts of coal dust. I may use plaster of paris or other calcium salts as the hardening cement, and I find that such material containing sulfur has 70 special advantages. In this case I use about 20 per cent. alcohol, 70 per cent. coal dust, 5 per cent. plaster of paris, and 5 per cent. water.

Should I wish to increase the degree of heat 75 as well as lasting qualities of my fuel in the plastic state I add petroleum to my mixture of alcohol and coal dust in the following proportions, 1 part of oil, 2 parts of alcohol, and 8 parts of coal dust. As however in this case 80 there is the tendency of the liquids to exude from the mixture before the degree of heat is sufficient to consume the entire mixture, I also mix therewith sawdust which readily absorbs the excess or exudation. The solid- 85 ity of the blocks or briquets aforementioned will be in proportion to the pressure applied, which in turn will also be determined or necessitated by the distance to which the blocks or bricks are to be trans- 90 ported. If it be proposed to burn the material near the place of manufacture, the proportion of binder or bond of union, as well as pressure, may be reduced, and hence the expense of production will to that degree 95 be also reduced.

In cases where I use petroleum as above indicated, I prefer to use crude petroleum, and it will be understood that its addition increases the plasticity of the mixture, and in 100 this instance I do not use cement but flour as a binder. The addition of sawdust by reason of its absorbent qualities aids in solidifying the material and renders it unnecessary to use so much flour or binding. Where petro- 105 leum is omitted and cement is used, or cement mixed with common clay, the binder is not combustible and this retards to a certain extent the combustion of the fuel produced, but on the other hand I secure the advantage of having a fuel which is more solid 110 and lasting.

While there are many cases in which it is preferable to use the alcohol and coal dust in the plastic state even with an excess of alcohol, yet there are other cases in which the 5 semi-plastic state is preferable, and in such cases I reduce the percentage of cement, or omit the cement entirely and mix with the said two prime elements a reduced percentage of common clay to the minimum at which it 10 does not reduce materially the desired rate of combustion.

It will be clear from what has been said above that my fuel may be manufactured at one point and shipped to various points 15 where it is to be used, or on the other hand the materials which are to enter into it may be shipped and the fuel actually manufactured at the place where it is to be used. It may be easily made in the form for immediate 20 use, and for this reason my combination of ingredients has special advantages.

In view of the fact that the whole combination which forms my fuel tends to absorb moisture I may mix with the material what 25 is known in the trade as japan, which is a widely known drier for paints and oils, and which is generally known as a mixture of shellac or other resin, metallic oxids, and turpentine. Instead of mixing this material 30 with the constituents of the fuel I may coat the blocks or bricks with it, and it will be understood that since japan is combustible it will add to the combustibility of the fuel as a whole. This japan coating is impervious 35 to moisture and thus protects the fuel. Instead of japan I may use pitch or artificial asphalt which is applied in melted form to the bricks or blocks, and it thus forms a coating 40 preventing the blocks from absorbing moisture, and also preventing the alcohol contained in the blocks from evaporating. In this case I use about 20 parts of alcohol, 70 parts of coal dust, 8 parts of cement, and 2 parts of pitch in 100 parts.

45 Where there is a scarcity of Portland cement I may use hydraulic cement or hydraulic lime either in its pure state or mixed with clay to reduce its cohesiveness to local or individual demands. Where hydraulic 50 cement is used the mixture would be about 1 part in 20, and where clay is added, about 1 part in 12.

I find that the addition of one per cent. of common salt (chlorid of sodium) improves 55 the fuel, and therefore I ordinarily add that amount during manufacture.

Having thus described my invention, what I claim and desire to secure by Letters Patent, is—

60 1. A solid fuel embodying a mixture of

coal dust and alcohol mixed in substantially the proportions of four to one.

2. A fuel embodying substantially one part alcohol, 4 parts coal dust and 1 part starch paste.

3. A fuel embodying alcohol, coal dust, starch paste and petroleum in substantially the proportions stated.

4. A fuel embodying alcohol, coal dust, starch paste, petroleum and common clay in 70 substantially the proportions stated.

5. A fuel embodying alcohol, coal dust, starch paste, petroleum, common clay and cement in substantially the proportions stated.

6. A fuel embodying alcohol, coal dust, petroleum, cement and common clay in substantially the proportions stated.

7. A fuel embodying alcohol, coal dust, cement and common clay in substantially the 80 proportions stated.

8. A fuel embodying alcohol, coal dust, petroleum, cement, common clay and sawdust in substantially the proportions stated.

9. A fuel embodying alcohol, coal dust, 85 sawdust, resin, petroleum, cement and common clay in substantially the proportions stated.

10. A fuel embodying alcohol, coal dust and hydraulic cement in substantially the 90 proportions stated.

11. A fuel embodying alcohol, coal dust, cement and flour in substantially the proportions stated.

12. A fuel embodying alcohol, coal dust, 95 an inert substance and salt in substantially the proportions stated.

13. A fuel embodying alcohol, coal dust and Portland cement in substantially the 100 proportions stated.

14. A fuel embodying alcohol, coal dust, petroleum and flour in substantially the proportions stated.

15. A fuel embodying alcohol, coal dust, cement and pitch in substantially the 105 proportions stated.

16. A fuel embodying a mixture of coal dust and alcohol mixed in substantially the proportions specified, and having a coating of combustible water-proof material.

17. A fuel embodying a mixture of coal dust and alcohol mixed in substantially the proportions specified, and having a coating of material known as japan.

In testimony whereof I affix my signature 115 in presence of two witnesses.

ALEXANDER H. EGE.

Witnesses:

W. H. RICE,

S. D. TAYLOR.